

No. 838,235.

PATENTED DEC. 11, 1906.

L. B. BUCHANAN.  
ELECTRIC FUSE.  
APPLICATION FILED APR. 2, 1906.

Fig. 1.



Fig. 2.



Fig. 3.

Witnesses:

H. B. Davis.  
Myrtina Doyle

Inventor:

Leonard B. Buchanan  
by Mayo & Hanninan

Atty.

# UNITED STATES PATENT OFFICE.

LEONARD B. BUCHANAN, OF WOBURN, MASSACHUSETTS.

## ELECTRIC FUSE.

No. 838,285.

Specification of Letters Patent.

Patented Dec. 11, 1906.

Application filed April 2, 1906. Serial No. 309,333.

*To all whom it may concern:*

Be it known that I, LEONARD B. BUCHANAN, of Woburn, county of Middlesex, State of Massachusetts, have invented an Improvement in Electric Fuses, of which the following description, in connection with the accompanying drawings, is a specification, like characters on the drawings representing like parts.

10 This invention relates to fuses of the so-called "cartridge" or "inclosed" type, one of which is disclosed in Letters Patent No. 801,467, granted to B. S. Luther and me, dated October 10, 1905, and may be used in 15 any fuse of the cartridge or inclosed type where a filling material is employed.

16 The object of my invention is to provide a fuse the sheath of which will be protected from an excessive rise in temperature, and 20 which will not explode or maintain an arc when the fuse-strip is disrupted, and which is not liable to deteriorate by exposure to dampness or lapse of time, and which may be made extremely sensitive so as to fuse with 25 great regularity on exposure for the requisite time to the prescribed overload.

17 I accomplish the object of my invention essentially by the use of a new and improved filling material.

30 Many filling materials have been suggested—for instance, silicic acid, slaked lime, plaster-of-paris, sand, ground asbestos, chimney-dust, ashes, slate-dust, calcium carbonate, and magnesium carbonate, all of 35 which have serious defects and operate unsatisfactorily. It is true that the probability of fire or injury to the apparatus by premature or delayed disruption of the fuse or heating or explosion of the sheath or otherwise may be much reduced or eliminated 40 when the defective filling materials hitherto used are employed by the use of fuses of larger dimensions than are necessary when my improved fuse is used or by the use of 45 expensive materials to protect the sheath from heat and other devices; but all of these devices add to the expense of the fuse and to the difficulty of manufacture and do not make the fuse less defective in principle, but 50 merely protect the apparatus in circuit with the fuse or the surroundings from the dangerous results of its defects.

Of the filling materials hitherto suggested sand, "set" plaster-of-paris, ground asbestos,

slaked lime, and slate-dust are unsatisfactory, 55 as the sheath heats to too high a temperature and the fuse operates too slowly. The carbonates of lime or magnesium (and unset plaster-of-paris if exposed to sufficient dampness) do not always prevent the explosion of 60 the fuse. In short, all previous fillings suggested have failed to produce perfect results and it is impossible to tell in advance by any knowledge of the physical and chemical properties of a material that it will operate 65 any better or even as well as a filling material as the materials hitherto used.

70 I have discovered that a filling material which meets all the requirements may be made from infusorial earth. The infusorial earth consists principally of silicic oxid. This is ordinarily mixed with considerable vegetable matter and traces of other substances. Unless the infusorial earth is reasonably free from clay and other non-volatile elements it should be treated in some manner, as by washing, to eliminate the clay, and by heating or otherwise to drive off the volatile materials. This treatment by heat should be at a temperature which will not 75 change the amorphous condition of silicic oxid. It will then be in a very fine powder and when applied as a filler in the usual way will make a very satisfactory filling material. The use with this filling material of a moderate 80 quantity of any of the filling materials now commonly used, such as slaked lime and plaster-of-paris, will not materially injure its operation; but I prefer to use the material alone. 85

90 Figure 1 shows in side elevation one form of electric fuse of the cartridge or inclosed type embodying my invention. Fig. 2 is a longitudinal section of the same, taken on the dotted line 2 2. Fig. 3 is an end view of the 95 fuse.

95 a represents the sheath or case of a fuse; b, the fuse-wire; c c, the terminals at the ends of the sheath or case; c' c', the end caps; d, the filling material which embodies my invention; e e, asbestos fiber or equivalent material, preferably tightly packed into the ends of the sheath or case; f f, packing rings or washers, and g g disks of paper or equivalent material. 100

105 The filling material d is practically pure silicic oxid derived from infusorial earth and produced by treating infusorial earth in such

manner as to substantially eliminate such clay and volatile elements as may be contained therein and not to modify or change the normal amorphous condition of the silicic 5 oxid therein.

Having thus described my invention; what I claim as new, and desire to secure by Letters Patent, is—

1. A fuse having a filling material consisting of amorphous silicic oxid, substantially as described.

2. A fuse having a filling material consisting of infusorial earth from which the clay and volatile elements have been substantially removed, substantially as described.

3. A fuse having a filling material consisting of infusorial earth from which the vola-

tile elements have been substantially removed, substantially as described.

4. A fuse having a filling material consisting of incinerated infusorial earth, substantially as described.

5. An inclosed fuse of the cartridge type having a filling material consisting of infusorial earth containing substantially only 25 amorphous silicic oxid, substantially as described.

In testimony whereof I have signed my name to this specification in the presence of two subscribing witnesses.

LEONARD B. BUCHANAN.

Witnesses:

B. J. NOYES,  
H. B. DAVIS.